

# UNITED STATES PATENT OFFICE.

HANS GOLDSCHMIDT, OF ESSEN-ON-THE-RUHR, GERMANY.

## ALLOY OF SILICON.

No. 921,607.

Specification of Letters Patent.

Patented May 11, 1909.

Original applications filed February 24, 1908, Serial No. 417,523, and April 24, 1908, Serial No. 428,933. Divided and this application filed January 19, 1909. Serial No. 473,044.

To all whom it may concern:

Be it known that I, HANS GOLDSCHMIDT, a subject of the King of Prussia, and resident of Essen-on-the-Ruhr, in the German Empire, have invented certain new and useful Alloys of Silicon, of which the following is a specification.

My invention relates to alloys of silicon with one of the alkali earth metals, calcium, 10 barium or strontium.

Calcium-silicon alloys have been produced at different times, but as far as commercial alloys are concerned which are to be manufactured on a large scale, these alloys were 15 always contaminated with carbon, as for instance the calcium-silicon prepared by Moissan. On account of such contamination the alloys always contained a smaller amount of the alkaline earth than they should contain 20 according to their theoretical composition.

The object of the present invention is to produce alloys of silicon with an alkaline earth metal which alloys are free from carbon and contain the alkali earth metal in 25 proportions up to 40 per cent. The processes by which these alloys are produced are described in my applications Serial No. 417523 filed February 24, 1908 and Serial No. 428933 filed April 24th, 1908 from which 30 the present application is a division. They are produced by heating silicon or ferro-silicon together with an excess of an oxid of the alkali earth metal in an electric or in a fuel heated furnace.

35 The alloy of silicon, for instance with calcium, according to the present invention may be produced as follows:—Two parts by weight of lime are mixed with one part by weight of silicon and the mixture is heated 40 to about the melting point of cast iron. The lime is in this way partially reduced and the liberated calcium forms with the silicon a calcium silicon alloy while the remainder of the lime forms a slag with the silicon. 45 This liquid slag may be regulated so that it crumbles on cooling and thereby enables the easy separation of the calcium silicon alloy. To aid this crumbling action a flux such as fluor spar is preferably added.

50 The heating of the mixture mentioned above may be effected either in an electric

or in a fuel-heated furnace and the proportions and ingredients may be modified as described in my copending applications Serial Nos. 417523 and 428933, from which 55 the present application has been divided out.

In the example given above where 2 parts of lime are treated with 1 part of silicon there results a calcium silicon alloy, which contains about 40% of calcium and is free 60 from carbon. These new alloys are used for aluminothermic purposes, and the calcium silicon alloy is especially useful also for the purpose of refining fused steel. The new alloys are specially adapted for this 65 latter purpose on account of their freedom from carbon, thereby preventing carbon from being newly introduced into the fused steel. Further the calcium silicon alloy has the effect of removing the last traces of 70 sulfur which may still be present in the fused steel. The calcium alloy according to the present invention has also the action of "killing" the steel and it forms a very fluid slag which soon mounts to the surface. 75 Further characteristics of the new alloys are, that they do not corrode when exposed to the air, that they may easily be crushed, that they are unaffected by water even when being placed under same, that they have a 80 metallic structure similar to silicon and exhibit a metallic sparkle when fractured.

I claim:

1. As a new product an alloy of silicon with an alkali earth metal which alloy is 85 free from carbon.

2. As a new product an alloy of silicon with an alkali earth metal which alloy is free from carbon and contains a considerable percentage of the alkali earth metal. 90

3. As a new product a calcium-silicon alloy free from carbon. 95

4. As a new product a calcium-silicon alloy free from carbon and containing up to 40 per cent. of calcium.

In testimony whereof I have hereunto set my hand in the presence of two witnesses.

HANS GOLDSCHMIDT. [L. S.]

Witnesses:

OTTO KÖNIG,  
WALTER E. KAMP.